

Nov. 4, 1958

H. A. TOULMIN, JR

2,859,150

METHOD OF MAKING TOWELS

Filed Oct. 18, 1955



INVENTOR  
HARRY A. TOULMIN, Jr.

BY

*Toulmin & Toulmin*

ATTORNEYS

2,859,150

**METHOD OF MAKING TOWELS**

Harry A. Toulmin, Jr., Dayton, Ohio, assignor to The Commonwealth Engineering Company of Ohio, Dayton, Ohio, a corporation of Ohio

Application October 18, 1955, Serial No. 541,262

5 Claims. (Cl. 154—76)

The present invention relates to paper towels, and more particularly to the manufacture of reinforced paper towels.

It is the principal object of this invention to provide an improved method of making reinforced paper towels.

It is a further object of this invention to provide a method of making paper towels by partially passing flock through a paper strip and securing the flock in position.

It is a further object of this invention to provide a method of making paper towels having tufts positioned perpendicular to both faces of a strip of paper.

It is an additional object of this invention to provide an improved paper towel.

It is still another object of this invention to provide a novel and simplified apparatus for the making of tufted paper towels.

Other objects and advantages of this invention will become apparent upon reference to the accompanying description when taken in conjunction with the following drawings wherein:

Figure 1 is a vertical sectional view of an apparatus for making paper towels in accordance with the teachings of this invention;

Figure 2 is a sectional view taken along the lines 2—2 of Figure 1;

Figure 3 is a sectional view taken along the lines 3—3 of Figure 1;

Figures 4 through 6 are partial vertical sectional views through the paper strip passing through the apparatus of Figure 1, showing the paper towel during various stages of the process; and

Figure 7 is a plan view of the reinforced paper towels made by the process of this invention.

The process disclosed by this invention essentially comprises moving a perforated paper strip through a chamber and evenly distributing a quantity of resin-treated flock upon the strip. The under surface of the strip is subjected to a vacuum to partially draw the flock through the perforations in the paper strip. The strip then progresses beneath electro-magnetic apparatus which establishes a magnetic field above the paper strip. The action of the magnetic field straightens the portions of the flock extending above the upper surface of the paper strip. The paper strip with the flock inserted therein and positioned substantially vertically to the strip is then passed through an oven to dry the resin and to secure the flock to the paper strip. The result is a reinforced tufted paper towel wherein the tufts extend away from the surfaces of the towel and do not lie flat against them.

To accomplish the method of this invention reference is made to Figure 1 wherein a container 1 contains a quantity of resin-treated flock indicated at 2. The flock consists of very short lengths of fabric refuse or vegetable or paper fibers. The fibers of flock are coated

with a thin film of a soft flexible resin binder to enable the flock to be firmly secured in the paper strip in a manner to be presently described.

Preferably a thermoplastic resin, such as glycerol-phthalic anhydride, is used. Also, a castor oil modified alkyd such as comprises 3 parts by weight alkyd resin and 1 part nitrocellulose provides a suitable soft flexible resin binder.

The chamber 1 has a dispensing opening 3 at the lower end thereof and a pair of cylinders 4 and 5 having longitudinally extending teeth thereon enmeshed with each other are mounted in the opening 3. The roller 4 has a shaft 6 extending outwardly of the chamber 1, as shown in Figure 2. A pulley 7 is mounted upon the end of the shaft 6 and is drivingly connected by a belt 8 to an electric motor 9.

The cylinders 4 and 5 rotate in the directions indicated by the arrows 10 and 11. This dispenses the flock between the rollers, as shown at 12 in Figures 1 and 2. The individual fibers of the flock are separated and are evenly distributed in a vertical plane, as shown in Figure 2.

The container 1 is mounted on the upper wall 13 of a chamber 14. The chamber 14 has end walls 15 and 16 each of which has openings 17 and 18 respectively therein. The bottom wall of the chamber 14 is indicated at 19 and slopes downwardly. There is an opening 20 at the lowermost portion of the bottom wall 19 and a conduit 21 attached thereto communicates with a vacuum pump 22.

Within the chamber 14 there is mounted an electro-magnetic apparatus indicated at 23 to establish a magnetic field adjacent the upper surface of the paper strip.

A paper strip, indicated at 24, and supported by a roller 25 is admitted through the opening 17 into the chamber 14.

Prior to the admission of the paper strip into the main chamber 14 a multitude of perforations are made over the entire surface of the paper strip. These perforations may be made by a mechanical device or by the distribution of drops of acid over the paper to form openings therein. As indicated in Figure 4, the openings or perforations to the paper strip are extremely small and extend across the entire width of the paper. The size of the openings is substantially equal to the diameter of the fibers constituting the flock.

The strip as it passes through the chamber 14 is supported by the bogey rollers 26 and 27. As shown in Figure 2, the chamber 14 is only slightly wider than the width of the paper strip 24.

Adjacent the end wall 16 of the chamber 14 there is located an oven, indicated at 28. A passage 29 communicates between the opening 18 and the oven 28. Electrical heating elements 30 and 31 are provided within the oven 28 and the paper strip passes between the heating elements, as illustrated in Figure 1, to enable both sides of the paper strip to be exposed to high temperatures.

In processing the paper strip in order to obtain tufted paper towels, the paper strip 24 is admitted to the opening 17 in the end wall 15 of the main chamber. As the paper strip passes beneath the flock container 1, flock indicated at 12 is evenly distributed upon the upper surface of the paper strip.

A sectional view through the paper strip 24 as it enters the main chamber 14 will reveal the condition of the paper to be as illustrated in Figure 4.

As the paper progresses past the flock container 1 it is exposed to the action of the vacuum pump 22 which creates a vacuum on the under surface of the strip. This vacuum draws ends of the flock fibers through the paper. The relationship of the diameters of the perforations and

fibers prevents the complete passage of the fibers through the perforations. As a result the flock only partially passes through the paper strip, with the end portions of the flock extending above both surfaces of the paper strip. The idler roller 26 at this point is vibrated both longitudinally and transversely to agitate the loose flock fibers upon the upper surface of the paper strip. In this manner, virtually all of the flock fibers will be drawn through the perforations under the action of the vacuum pump 22.

At this stage of the process a section through the paper strip 24 will reveal the condition of the paper as illustrated in Figure 5. In Figure 5 the individual flock fibers, as indicated at 33, have their lower portions 34 extending straight downwardly under the action of the vacuum pump 22. The upper ends of the flock fibers, as indicated at 35, are flat upon the upper surface of the paper strip. This is also partially due to the action of the vacuum pump 22.

The paper strip 24 with the flock fibers partially inserted therethrough is then passed beneath the electro-magnetic apparatus 23 and the magnetic field created thereby. The action of the magnetic field upon the fibers causes the upper portions 35 of the fibers to straighten, as indicated in Figure 6. Consequently, after the strip emerges from beneath the electro-magnetic apparatus 23, the flock fibers have both end portions substantially perpendicular to the surfaces of the paper strip 24.

With the fibers straightened by the action of the electro-magnetic apparatus 23, the paper strip is then passed through the opening 18 into the drying or baking oven 28. The heat of the heating elements 30 and 31 dries the solvents from the resin and secures the flexible flock fibers within the perforations in the paper strip.

Upon emerging from the drying oven the process is completed. The result is a reinforced tufted paper towel of which a plan view would be as illustrated in Figure 7. The resulting paper towel has greater strength because of the reinforcing action of the flock and the resin. In addition, the drying properties of the towel are greatly increased because of the presence of the flock tufts over both surfaces of the paper towel.

The towel fabricated by this process may be also used as disposable paper material such as handkerchiefs, wipers for industry and the like.

It will be understood that this invention is susceptible to modification in order to adapt it to different usages

and conditions, and, accordingly, it is desired to comprehend such modification within this invention as may fall within the scope of the appended claims.

What is claimed is:

1. In a method of making tufted paper towels, distributing flock over a perforated paper strip, subjecting individual lengths of flock to an air stream to insert the flock in the perforations to extend above both faces of the paper, and securing the flock in the strip.

2. In a method of making tufted paper towels, perforating a strip of paper with holes evenly distributed thereover, coating lengths of individual fabric fibers having diameters substantially equal to the diameter of said holes with a resin, establishing air streams through the holes in the paper to propel the resin-coated fabric fibers into said holes whereby the resin will prevent the passage of the fibers completely through the holes and the ends of each fiber will protrude above the surfaces of the paper strip, and heating the resin to secure the fibers in the paper strip.

3. In a method of making towels, the steps of applying a vacuum to the underside of a perforated sheet, and distributing a plurality of individual lengths of fibers above the perforated sheet to thrust single fibers in said perforations under the action of the vacuum effected through the perforations.

4. In a method of making paper towels, the step of perforating a sheet of paper, distributing a plurality of individual lengths of fibers above the perforated sheet, establishing air streams through said perforations to propel said fibers into said perforations, and securing said fibers within said perforations so that both ends of said fibers project above the surfaces of the sheet.

5. A paper towel comprising a perforated sheet of paper, a single fabric fiber in each of said perforations and extending above both faces of said sheet, and a resinous coating on each fiber which when hardened will secure the fibers in said perforations.

#### References Cited in the file of this patent

#### UNITED STATES PATENTS

|           |              |               |
|-----------|--------------|---------------|
| 527,971   | Grubb        | Oct. 23, 1894 |
| 1,810,328 | Slater       | June 16, 1931 |
| 1,831,064 | Frederick    | Nov. 10, 1931 |
| 2,715,074 | Hirschburger | Aug. 9, 1955  |